

H. A. GARDNER,  
FABRIC FOR AIRSHIPS AND PROCESS OF MAKING SAME,  
APPLICATION FILED JAN. 6, 1920.

1,381,413.

Patented June 14, 1921.



Inventor

*H. A. Gardner*

By

*R. A. Blair*

Attorney

# UNITED STATES PATENT OFFICE.

HENRY A. GARDNER, OF WASHINGTON, DISTRICT OF COLUMBIA.

## FABRIC FOR AIRSHIPS AND PROCESS OF MAKING SAME.

1,381,413.

Specification of Letters Patent. Patented June 14, 1921.

Application filed January 6, 1920. Serial No. 349,837.

To all whom it may concern:

Be it known that I, HENRY A. GARDNER, a citizen of the United States, residing at Washington, District of Columbia, have 5 invented new and useful Improvements in Fabrics for Airships and Processes of Making Same, (Case C,) of which the following is a specification.

This invention relates to outer envelop 10 fabric for rigid airships and process of making the same and an object of the invention is to produce a fabric which will not deteriorate on exposure to the action of light and heat.

15 Another object of the invention is to produce a strong, durable fabric which is water-proof and fire-proof and possesses a high tensile strength.

20 A further object of the invention is to provide a novel process of manufacture of the fabric.

25 For the protection of the gas cells and the aluminum strength members that are used in rigid airships, an outer cover consisting of cloth to which dope has been applied to render it water resisting, has heretofore been used. This cloth, however, is more or less inflammable and, because of the contributing effect of the dope, becomes rotted on 30 exposure to the light for any extended period of time.

35 In my process I have produced a rigid cover having distinct advantage over that previously produced for this purpose. For the manufacture of this fabric, I usually select as the base a high strength, high count cotton of the following construction:

|                              |            |
|------------------------------|------------|
| Weight per square yard       | 2 ounces.  |
| Width                        | 38 inches. |
| 40 Minimum tensile strength: |            |
| Warp                         | 35 lbs.    |
| Filling                      | 35 lbs.    |
| 45 Minimum thread count:     |            |
| Warp                         | 116 lbs.   |
| Filling                      | 124 lbs.   |
| 50 Yarn size:                |            |
| Warp                         | 80 lbs.    |
| Filling                      | 85 lbs.    |

50 The drawing is a sectional view of a portion of fabric made in accordance with my invention illustrating diagrammatically the arrangement of the substance or material applied thereto.

The cloth 10 is first rendered fire resisting 55 by treatment with a 10% aqueous solution of ammonium phosphate brought to a temperature of approximately 150° F. The cloth automatically passes through this solution and then through a series of rolls to remove 60 the excess and then out onto a tenter frame over a series of steam coils to be dried. During drying, the cloth may be made as taut as desired, in order to prevent wrinkling and other defects. The use of the above 65 mentioned fire resisting salt I do not claim as novel. I may, however, add to the ammonium phosphate solution from 2% to 10% by weight of a pigment such as red iron oxid or carbon black; the purpose being 70 to stop the light rays which affect the strength of the fabric. The cloth is usually dry at the end of ten minutes, at which time it is rolled on a mandrel and put through the second treatment which consists of the application of a very thin coat of cellulose dope 75 containing, if desired, a small percentage of treated tung oil which forms a film 11 on both sides of the cloth 10. I may, if desired, add to the dope from 2% to 10% of pigment such as iron oxid or carbon black, the purpose being to stop the light rays which affect the strength of the fabric. The cloth then passes onto the tenter frame 80 and is then dried under tension. I studiously avoid the use of linseed oil or other vegetable oils which dry by oxidation, since their use may develop acid products that seriously injure cotton when exposed to the atmosphere or even when stored. On the other hand, tung oil dries largely through polymerization 85 and produces a film that does not react with the fabric. By the above process there is produced a fire resisting fabric having high tensile strength and a water shedding surface. The fabric being impregnated with waterproofing is resistant to moisture on both sides and is not subject to loss of tension by absorption of moisture, 90 as is the type of fabric now in use.

When this fabric is placed over a rigid ship and laced in place, one or more additional coats of dope containing aluminum powder are applied forming a film 12 on the outside thereof. Great tautness is obtained 105 and a surface of high solar radiation is produced. With such a fabric the gas in the cells of the ship will remain at a temperature

from 20° to 30° lower than when covered with the ordinary dark or untreated colored fabric. Due to the high light reflecting surface of the fabric, the cloth remains strong 5 for a long period of time.

It will be understood that the process of manufacture may be varied in unessential particulars, and that equivalent ingredients may be used in the place of the ones mentioned without departure from the principles of the invention. I do not restrict myself to precise proportions of materials or to other unessential limitations but contemplate such variations as are within the 15 principles of the invention as set forth in the appended claims.

What I claim is:

1. A fabric of the class described comprising a cloth base treated with a suitable fireproofing compound and a film containing an oil of the class which dries by polymerization.
2. A fabric as set forth in claim 1, and a second film containing an oil of the class which dries by polymerization.
3. A fabric as set forth in claim 1, said film comprising cellulose dope containing an oil of the class which dries by polymerization.
- 30 4. A fabric as set forth in claim 2, said second film comprising a cellulose dope containing an oil of the class which dries by polymerization.
5. A fabric as set forth in claim 3 and a second film on said first named film comprising a cellulose dope containing an oil of the class which dries by polymerization.
- 40 6. A fabric of the class described comprising a cloth base treated with a suitable fireproofing compound and a film of cellulose dope containing tung oil.
7. A fabric as set forth in claim 6 and a second film of cellulose dope containing tung oil.
- 45 8. A fabric as set forth in claim 7, said second film containing finely divided aluminum powder.
9. A fabric as set forth in claim 8, said second named film containing 10% finely divided aluminum powder.
- 50 10. A fabric of the class described comprising a cloth base treated with a suitable fireproofing compound, a film containing an oil of the class which dries by polymerization and a second film on said first named film containing finely divided aluminum

powder and an oil of the class which dries by polymerization.

11. The process of making fabric of the class described which consists in treating a 60 cloth base with a fireproofing solution, delivering said base through a series of rolls to remove excess solution, and coating said cloth base with a dope containing an oil of the class which dries by polymerization. 65

12. The process as set forth in claim 11 including the application of a second coating of dope containing an oil of the class which dries by polymerization.

13. The process as set forth in claim 11 70 including subjection of the cloth base to heat and tension prior to applying the coating of dope.

14. The process as set forth in claim 12 75 wherein the fabric is laced in place over a rigid airship prior to the application of said second named coating of dope.

15. The process as set forth in claim 12, said second named coating of dope containing 80 finely divided aluminum powder.

16. The process as set forth in claim 15, said second named coating of dope containing 10% finely divided aluminum powder.

17. The process as set forth in claim 15, including subjection of the fabric to heat 85 and tension prior to the application of said second named coating of dope.

18. The process of making a fabric of the class described which consists in treating a cloth base with a fireproofing solution, delivering said base through a series of rolls to remove excess solution and coating said cloth base with a dope containing cellulose and tung oil. 90

19. The process as set forth in claim 18, 95 including the application of a second coating of dope containing cellulose and tung oil.

20. The process as set forth in claim 19 including subjection of the fabric to heat and tension prior to the application of said 100 second coating of dope.

21. The process as set forth in claim 19, said second named coating of dope containing finely divided aluminum powder.

22. The process as set forth in claim 19 105 wherein the fabric is laced in place over a rigid airship prior to the application of said second named coating of dope.

Signed at Washington, District of Columbia, this 3d day of December, 1919. 110

HENRY A. GARDNER.